

(No Model.)

W. E. COREY & F. L. SLOCUM.

PROCESS OF MAKING CARBONIZED STEEL FOR ARMOR PLATES.

No. 574,668.

Patented Jan. 5, 1897.



WITNESSES

*J. P. M. Corwin*

INVENTORS

Frank Leroy Slocum  
William Ellis Corey  
by Beulah Belknap  
their atto

# UNITED STATES PATENT OFFICE.

WILLIAM ELLIS COREY, OF MUNHALL, AND FRANK LEROY SLOCUM, OF PITTSBURG, PENNSYLVANIA, ASSIGNORS TO THE CARNEGIE STEEL COMPANY, LIMITED, OF PITTSBURG, PENNSYLVANIA.

## PROCESS OF MAKING CARBONIZED STEEL FOR ARMOR-PLATES.

SPECIFICATION forming part of Letters Patent No. 574,668, dated January 5, 1897.

Application filed May 28, 1896. Serial No. 593,429. (No specimens.)

*To all whom it may concern:*

Be it known that we, WILLIAM ELLIS COREY, of Munhall, and FRANK LEROY SLOCUM, of Pittsburgh, in the county of Allegheny and 5 State of Pennsylvania, have invented a new and useful Improvement in Methods of Making Carbonized Steel for Armor-Plates, of which the following is a full, clear, and exact description, reference being had to the accompanying drawing, which shows in longitudinal section apparatus adapted for the practice of our invention.

Our invention relates to the supercarburization of plates or pieces of steel of any size 15 or description, but is specially designed to be applied in the manufacture of large plates or masses of steel to be forged or otherwise shaped into armor-plate.

Steel for the manufacture of armor-plates 20 is usually made by first manufacturing the steel in any of the usual methods, but preferably by converting cast-iron into steel in the hearth of a furnace by the method known as the "open-hearth" process. The steel so 25 manufactured may be alloyed with nickel, with addition of manganese, spiegeleisen, aluminum, or other metallic ingredient; and our invention is applicable to steel manufactured by any suitable process and of any desired 30 composition of ingredients, containing such amount of carbon as may be desired, that is, the steel, before subjecting it to supercarburization, (as in the case of armor-plate,) should receive a certain percentage of carbon while 35 in the furnace and before pouring, so that an increased amount of carbon may be added on one side of the plate by the process known as "supercarburization," which renders the finished plate extremely hard on one face, while 40 it is much softer on the other face, the degree of carbon gradually increasing from the soft to the hard side, which effect has for many years been known to be the necessary result of cementation applied to one side only of a 45 plate or mass of iron or steel, while the other side is protected from the external application of the carburizing agent.

In the recarburizing, or, as it is termed more properly, the "supercarburizing," of steel, 50 and especially in the manufacture of armor-

plate, it is desirable to use a sufficient degree of heat, preferably below that of the melting-point of cast-iron, and especially so because a high degree of heat is very injurious to the quality of the steel.

Our improvement is based upon the discovery which we have made that steel plates can be supercarburized very rapidly and with improved results by heating the same with the surface to be supercarburized in contact 55 with calcium carbid. The calcium carbid is a convenient and easily manageable reagent for the purpose. It acts much more rapidly than does free carbon in the form of charcoal, and its action on the steel is readily controllable.

The steel, having been manufactured in a suitable furnace (such, for example, as an open-hearth furnace) containing the ordinary amount, say one-fourth of one per cent., 60 of carbon, is cast into an ingot of suitable dimensions and then rolled or otherwise shaped into a plate of the desired form. This plate is then placed in a suitable heating-furnace, 65 preferably a gas-furnace of suitable construction, within a suitable receptacle with refractory lining of such dimensions as to receive the steel plate and permit the application of carburizing and protecting agents. On the bed of this receptacle is placed a layer 70 of ground or pulverized calcium carbid of suitable depth, depending on the thickness of the steel plate under treatment. A layer containing carbid of six to eight inches in depth will suffice for a steel plate of from ten 75 to fifteen inches in thickness, and on this layer of carbid is laid the steel plate.

The plate may be introduced into the furnace and deposited on the layer of calcium carbid either when the plate is cooled or, if preferred, 80 when preheated to about 1,800° Fahrenheit. The plate or plates are preferably in a horizontal position, as being more convenient when the carbid is in comminuted form. On the top and around the steel plate is placed 85 sand or other suitable protecting material. The receptacle thus charged is then exposed to a gradually-increasing heat in the furnace, 90 on the hearth of which the receptacle may be permanently or removably situated. The 95 100

heat is gradually increased until the requisite temperature is obtained, which should be from 1,800° to 2,100° Fahrenheit, it being necessary to raise the steel plate under treatment to a high temperature in order to enable it to absorb the additional amount of carbon required to supercarburize the steel plate. The temperature stated should be maintained in the furnace for, say, six days of twenty-four hours each, more or less, depending on the thickness of the mass of steel to be supercarburized. The heat is then gradually reduced during a further period of five days until it reaches a temperature of about 1,400° Fahrenheit, when the plate is removed from the furnace. Several steel plates may be placed in the furnace at once with layers of the carbid between the surfaces to be supercarburized.

In the accompanying drawing we show apparatus which is well adapted to the practice of our invention. Our claim, however, is not limited to the construction of the apparatus, but refers to the method herein described.

In the drawing, 2 is the heating-furnace, having ranges of gas-ports *a* and *b* on each side, through which the heating-gas is introduced on one side of the furnace and out of which it passes on the other. The direction of the gas may be reversed from time to time. The movable hearth *B* is carried upon a truck *C*, mounted on wheels *w*, and is adapted to be moved into and out of the heating-chamber by means of a motor-cylinder *d*. This hearth *B* consists of a horizontal bed *e*, of brick or other refractory material, below the surface of which and extending across the hearth are flues *c c*, which are at such height as to coincide with the lower range of gas-ports *a* in the furnace, while the upper range of gas-ports *b* are at or about the level of the upper surface of the upper armor-plate *D*. By this arrangement the heating-gas passes through the upper and lower ports *a b* on one side, passing through the flues under the hearth or bed *B* and over the top of the upper plate, whereby the furnace is suitably heated to the degree requisite or desired for treating the armor-plates, the heating-gas being supplied in the usual manner to the furnace from a generator outside.

At each end of the bed *e* of the hearth is built a temporary wall *f*, of such shape and size as to fit into and close the open ends of the furnace. From each side of the movable hearth *B* there projects an inclined flange *g*, of iron, which, when the truck *C*, carrying the movable hearth, is run into the furnace, fits

against an inclined projection *h h* from the bottom of the inner wall of the furnace, thus closing the heating-chamber on both sides as well as at the ends.

The armor-plates *D E* to be supercarburized are placed in the hearth of the furnace with a layer *F* of comminuted calcium carbid between the surfaces to be supercarburized, and the carbid is protected from oxidation preferably by incasing the edges of the plates in sand *k*.

Other apparatus may be used for heating the armor-plates to be carburized on one side, and, if desired, one plate only at a time may be treated, or a series of plates may be treated in the furnace at the same time by making obvious changes in the apparatus, which we have described in this specification not for the purpose of basing any claims thereon, but for the purpose of illustrating a practical method of using our improved process.

The special advantages resulting from the use of our improvement are due to the employment of the highly-active calcium carbid, the carbon of which unites with the steel much more rapidly and efficiently than when the carburization or supercarburization of steel is effected by the ordinary processes involving the employment of animal or vegetable charcoal, or of mineral carbon, or of hydrocarbon vapor, as of petroleum, or of the ordinary coal-gas, so that whereas in the process as heretofore practiced the time required for supercarburizing a steel armor-plate was about twenty-seven days, or six hundred and forty-eight hours, it can be done by our process in fifteen days, or three hundred and sixty hours.

We desire to include as equivalents under the term "calcium carbid" similar metallic carbids, such as the double carbid of magnesium and calcium.

We claim—

The process herein described for supercarburizing steel for armor-plates and other purposes, which consists in heating the same with the surface to be supercarburized in contact with calcium carbid.

In testimony whereof we have hereunto set our hands.

WILLIAM ELLIS COREY.  
FRANK LEROY SLOCUM.

Witnesses as to W. E. Corey:

W. H. CORBETT,  
L. C. EAKMAN.

Witnesses as to F. L. Slocum:

G. I. HOLDSHIP,  
H. M. CORWIN.